

Patented June 26, 1928.

1,674,957

# UNITED STATES PATENT OFFICE.

REGINALD SCOTT DEAN AND WILLIAM EWART HUDSON, OF OAK PARK, ILLINOIS, AS-  
SIGNORS TO WESTERN ELECTRIC COMPANY, INCORPORATED, OF NEW YORK, N. Y.,  
A CORPORATION OF NEW YORK.

## PROCESS FOR IMPROVING LEAD-ALLOY ARTICLES.

No Drawing.

Application filed February 5, 1924. Serial No. 690,719.

This invention relates to a process for improving lead alloy articles, particularly lead alloy articles on which work has been performed.

5 An object of this invention is to provide a process for improving articles which have been formed from certain lead alloys.

A further object of this invention is to provide a process for so forming lead alloys 10 that the process of improving and forming may be carried out substantially at the same time.

A further object of this invention is to provide a process for forming articles from 15 a hardened sheet of lead alloy.

The process may be used to advantage in the manufacture of various products made of an improved lead alloy and particularly in the manufacture of storage battery plates 20 and improved lead alloy tape.

Heretofore articles formed from lead or lead alloys have been insusceptible to hardening except by the simple addition of matter, which would have the effect of forming 25 with the lead an alloy which would be somewhat harder than the lead. A process has been worked out which makes possible a considerable hardening and improving of lead by the addition of a small percentage 30 of antimony or other alloying element, such as tin, and a subsequent heat treatment. For a full disclosure of the details of this treatment, reference is made to our co-pending application, Serial No. 690,716, filed February 5, 1924.

It is sufficient to state here, briefly, that this heat treatment consists in adding to lead, matter the solubility of which in lead varies with temperature, reducing the resulting alloy to a solid solution forming a supersaturated solid solution, and allowing the alloy to assume a more stable state. One process for accomplishing these objects is described in our application above referred to, which process consists briefly in heating, 45 quenching and aging the alloy.

This invention is based on the discovery that the formation of a lead alloy solid solution can be brought about more quickly 50 when work is performed upon the alloy article, thereby greatly reducing the time required in the heating step of the process described in the application referred to

above. The time that would be required for heating is materially cut down because the work which is performed upon the alloy has the effect of breaking down the structural formation of the mass and reducing it to such a state that the solution takes place very quickly. A lead alloy article if heated 55 to a temperature required to obtain a solid solution of the particular elements present may be reduced to a homogeneous solid solution almost instantaneously by any work violent enough to cause deformation of the 60 crystalline structure. In the case, for instance, of an alloy having approximately 2½ per cent antimony to 97½ per cent lead, heated to a temperature of 240° C. and 65 rolled or struck with a machine hammer or punch or other forming tool, solid solution is formed quickly enough so that immediately after the work has been completed, the article may be quenched in any convenient 70 way to a temperature below 100° C. After this quenching, aging at room temperature or at temperatures below 100° C. will cause 75 a very great hardening and improvement of the alloy.

In our co-pending application referred to 80 above it is shown that the time of heating required for a cast lead antimony article of 2.25% antimony content is about seventy-two hours. As noted also in this application work performed upon the lead antimony article tends to hasten the forming of 85 solution. All other variables i. e. temperature, percentage of solute and the like, being equal the time of heating is cut down, proportionally to the work performed. 90 When a very great amount of work is exerted on the alloy a substantially solid solution can sometimes be formed in only a few minutes.

The type of work may vary, and the results remain substantially the same.

The method constituting the present invention may be employed to advantage where antimony is used as the alloying element and the article formed from the alloy is stamped out cold, or if it is stamped out hot must be allowed to cool for some reason. This formed article in its cold state may be heated up to the temperature which would be required for the antimony present to enter solution. It will be found that only a 100 105

comparatively small amount of time is required then for a solid solution to form at the given temperature. The article may then be quenched and aged in the manner set forth in our co-pending application above referred to. It will be found that articles which have been formed for two or three years may be hardened under this method in a very short length of time, providing said article has, during this period, remained at a temperature below the temperature of recrystallization of the alloy constituents, believed in lead antimony alloys of the type employed to be about 100° C. If this article has, during this period of time, been at a higher temperature, so as to permit recrystallization, the time required for heating must be considerably lengthened.

20 A suitable illustrative process which can be adapted to the manufacture of articles which can be formed by rolling is as follows:— The proper proportions of lead and alloying element may be cast in the form 25 of an ingot and heated to a temperature slightly below the fusing temperature. The ingot is then rolled into the form required and kept hot during this rolling process. Upon coming out of the rolls it is quenched 30 and aged at room temperature. Such a process can be applied to the manufacture of lead alloy tape and similar articles.

As a further illustration a process to be used for forming lead alloy articles such 35 as storage battery grids by means of stamping machinery, may be carried on in the following manner:

The lead alloy is cast into the form of an ingot and heated when solid to a temperature of about 240° C. It is then introduced hot into a set of rolls where it is rolled into the form of a flat sheet. This flat sheet is introduced hot under the stamping machinery and the form required stamped 45 therefrom. The formed article is then quenched and aged at room temperature.

Such a process for forming lead alloy articles by means of stamping machinery

and the like may also be carried on as follows:

The lead alloy is cast in requisite proportions in the form of a slug or ingot. The said ingot is then heated to a temperature below the fusing temperature and introduced at that temperature into a set of rolls 55 where it is rolled into the form of a flat sheet. The flat sheet is quenched as it comes from the rolls and allowed to harden by aging at room temperature. Either before or after the sheet has attained maximum 60 hardness the desired forms may be stamped therefrom. Whatever the type of work employed the article may be quenched immediately after the forming of the solid solution. If the work at the high temperature has not 65 been sufficient to form the solution, additional heating will be required before the article is quenched.

What is claimed is:

1. A process for producing improved 70 formed articles composed of a lead-antimony alloy, which consists in casting a lead-antimony ingot with an antimony content up to three per cent, rolling said ingot at a temperature below 245° C. to form a solid solution 75 of the alloy and to work the ingot into the shape required, quenching said rolled article to a temperature below 100° C. to produce a supersaturated solid solution, and aging at a temperature below 100° C. 80

2. A process for producing improved formed articles composed of a lead-antimony alloy, which consists in casting the lead-antimony alloy in the form of an ingot, rolling said ingot while hot to form a solid solution 85 of the alloy and to shape the ingot into a sheet, stamping said article from the sheet, quenching to a temperature below 100° C. to produce a supersaturated solid solution, and aging at a temperature below 100° C. 90

In witness whereof, we hereunto subscribe our names this 22nd day of January A. D., 1924.

REGINALD SCOTT DEAN.  
WILLIAM EWART HUDSON.